

# UNITED STATES PATENT OFFICE.

GEORGE W. MILES, OF BELMONT, MASSACHUSETTS, ASSIGNOR TO ROSS CHEMICAL COMPANY, OF BOSTON, MASSACHUSETTS, A CORPORATION OF MAINE.

## METHOD OF INCORPORATING FILLING MATERIAL IN PAPER.

1,228,580.

Specification of Letters Patent.

Patented June 5, 1917.

No Drawing.

Application filed March 11, 1915. Serial No. 13,692.

*To all whom it may concern:*

Be it known that I, GEORGE W. MILES, a citizen of the United States, and resident of Belmont, in the county of Middlesex and 5 State of Massachusetts, have invented new and useful Improvements in Methods of Incorporating Filling Material in Paper, of which the following is a specification.

My invention relates to the manufacture 10 of filled paper and consists in a novel method of introducing filling or coating material, such as china clay, blanc-fixe, satin white, or any of the finely comminuted mineral fillers which are habitually incorporated in the 15 paper, and also in the product which results from the practice of my new method.

Heretofore paper manufacturers have incorporated limited amounts of filler, such as china clay, with the pulp before it passes to 20 the paper web-making machine. By the practice heretofore prevailing the fiber will carry only a limited amount of clay or other filler, the maximum proportion being about twenty-five per cent. by weight of the finished paper web. Where larger amounts of 25 filler than could be incorporated with the pulp have been desired, such as for the production of paper for half tone work, the additional amount in processes at present in 30 vogue must be applied to the surface of the paper web, whereas by my new process herein to be described the paper as it comes from the web-forming machine carries a sufficient amount of filler to be suitable for half tone 35 work.

I have discovered that if an emulsion of 40 wax or waxy material such as stearic acid is introduced into the beater with the fiber together with a filler such as china clay, the effect of the wax is to carry into association 45 with the fiber a much larger proportion of the filler than can otherwise be incorporated with it. By way of preferred modification of this treatment, I also add a size, such as rosin size. Moreover, I prefer, and recommend the use of, an emulsion of paraffin wax for this purpose. Paraffin wax can be emulsified by a process which I have described and claimed in my United States Patent, 50 No. 1,168,534, dated January 18, 1916. Briefly described, this emulsification process is as follows:

Take of paraffin wax ninety-five parts, and of commercially dry soda tallow soap 55 (containing about 20% water) five parts, by

weight. Make a paste with the soap in from four to five times its weight of water. Then melt the paraffin wax and stir the paste into it, heat approximately to the boiling point of water and maintain the heat, meanwhile 60 stirring or beating until, by evaporation, the water is reduced to that critical proportion which effectuates the emulsification of the wax. The emulsion thus formed is quite thick, and may with advantage be extended 65 by the addition of more water.

The introduction of such a wax emulsion into the pulp has this effect: that proportions of size—such as rosin size—much larger than heretofore possible can be employed, without incurring the detriment of foaming and sliming at any stage of the paper manufacture. While the introduction and use of the wax emulsion alone will enable the manufacturer to incorporate with 70 the fiber a larger proportion of filling material—such as china clay—than heretofore, the employment of a size such as rosin size, in association with the wax emulsion will enable him to carry even larger proportions 75 of filler with the fiber, and, with increase in the proportion of size (made practically possible by the presence of wax emulsion) the proportion of filler may be increased to any extent within practical limits. 80

For example: To 200 parts (by weight) of wet paper stock (containing about 44 parts bone dry fiber, by weight) add 2 parts rosin in soap form, and 5 parts paraffin wax in emulsion, and 50 parts china clay, and 85 agitate these ingredients in the beater. Test of the back water indicates the presence therein of about 2.25 parts china clay. With the exception of this small proportion remaining in the back water, the china clay is 90 carried with the fiber, wax, and size, into the paper body. The treatment of the stock and the manufacture of the paper web, is carried out in the usual way, the size being precipitated with alum or the like. The paper thus produced, on being compacted or calendered, presents an excellent surface for printing or for the reception of half tone process prints. 95

By the above described process, filled paper can be produced which is suitable for many purposes for which heretofore coating of the finished paper web has been necessary.

I claim:

1. A method of incorporating filling ma-

terial in paper, which consists in mixing with the fiber before its final formation into a paper web an emulsion of waxy material with a proportion of filler in excess of that which in the absence of said emulsion will incorporate with the fiber.

2. A method of incorporating filling material in paper, which consists in mixing with the fiber before its final formation into a paper web an emulsion of paraffin wax with a proportion of filler in excess of that which in the absence of said emulsion will incorporate with the fiber.

3. A method of incorporating filling material in paper which consists of mixing with the fiber in the beater an emulsion of

waxy material with a proportion of filler in excess of that which in the absence of said emulsion will incorporate with the fiber.

4. A method of incorporating filling material in paper which consists in mixing with the fiber in the beater an emulsion of paraffin wax with a proportion of filler in excess of that which in the absence of said emulsion will incorporate with the fiber. 20 25

Signed by me at Boston, Massachusetts, this 5th day of March 1915.

GEORGE W. MILES.

Witnesses:

ROBERT CUSHMAN,

CHARLES D. WOODBERRY.